

# UNITED STATES PATENT OFFICE.

CARLETON ELLIS, OF LARCHMONT, NEW YORK, ASSIGNOR, BY MESNE ASSIGNMENTS,  
TO COPPER OIL PRODUCTS COMPANY, A CORPORATION OF NEW YORK.

## PROCESS OF PRESERVING WOOD AND PRODUCTS THEREOF.

1,054,756.

Specification of Letters Patent.

Patented Mar. 4, 1913.

No Drawing.

Application filed January 27, 1909. Serial No. 474,565.

To all whom it may concern:

Be it known that I, CARLETON ELLIS, a citizen of the United States, residing at Larchmont, in the county of Westchester 5 and State of New York, have invented certain new and useful Improvements in Processes of Preserving Wood and Products Thereof, of which the following is a specification.

- 10 This invention relates to processes of preserving wood and products thereof; and it comprises a method of preserving wood by impregnating the same with a heavy asphaltic oil carrying a dissolved fungicide; and 15 it also comprises wood impregnated and preserved by a contained asphalt-like body carrying a dissolved fungicidal mineral body; all as more fully hereinafter set forth and as claimed.
- 20 In the rotting, decay and perishing of wood and like materials, a number of factors are active, but air and moisture must both be present. Part of the decay is due to bacteria and part to the higher fungi such 25 as those producing dry rot. In the prior art a number of materials have been used for the purpose of preserving the wood but none of these serves the purpose intended as well as can be desired. Oily bodies, such as "creosote" (coal tar preparations), and other thin oily preparations have been used for saturating wood, their activity largely depending upon their power of excluding air. 30 These preparations however have no active fungicidal value against the higher fungi, though they contain more or less of the phenols which are antiseptic against the lower fungi such as the bacteria. In so far as they contain phenols however, they exercise 35 a detrimental action upon the fiber, phenols "softening" or tendering fiber. Preservation is sometimes done with inorganic toxic bodies such as corrosive sublimate, zinc chlorid, and the like. These bodies in so far 40 as they are soluble do not remain in the wood but tend to leach out while if insoluble their preservative action is very little. Insoluble bodies in the wood have also the disadvantage of lessening its mechanical 45 strength. Another objection to thin oils is the fact that they are apt to be lost by capillary exchange where the wood is in contact with the soil, as in ties and the like. A tie treated with a liquid preservative and

in contact with dry soil tends to lose its 55 preservative, the liquid averaging itself between the two capillary bodies, the timber and the soil. In the course of time this action being continued, the thin oil tends to be lost wholly or in large part. And the 60 phenols, which are the only antiseptic bodies of the "creosotes" are more or less volatile and soluble so that they disappear in time.

A wood preservative for such purposes as treating ties, piles, telegraph and telephone 65 poles, and the like, must have a number of properties which it is hard to find combined in a single material. It must be relatively soft, fluent or plastic so that it may not interfere with the mutual relations of the 70 wood fibers; it must be relatively thick when cold so that it may not be extracted from the wood by capillary action; it must be wholly insoluble that it be not extracted from the wood by penetrating moisture; it must be 75 wholly non-volatile, and it must have active fungicidal and bactericidal properties. Such a material, however, I can provide by the simple expedient of dissolving fungicidal mineral matter in an asphalt-like substance. 80 With the proper grade of asphalt or asphalt-like oil the impregnating body fulfils all the physical requirements, not injuring the fiber of the wood, not volatilizing, not dissolving, and not being extracted by seepage or capillary action. Such an asphalt or asphalt-like oil, however, while desirable in these respects has little or no positive bactericidal or fungicidal action, except in so far as it contains sulfur compounds. This property 85 may be imparted to it by dissolving therein suitable fungicidal or bactericidal substances. While various organic fungicides such as Martius yellow (a sodium salt of 2,4, dinitro-a-naphthol) or the like may be 90 used, I much prefer a substance containing a fungotoxic metallic oxid or compound. The compounds of the metals are not usually soluble in organic solvents such as asphalt but by combining the metallic oxid with a suitable oily or organic acid or a plurality of such acids, compositions may be obtained 95 which are so soluble. As such a soluble salt I preferably use an oleate or palmitate of copper, through phenolates, resinates and 100 many other salts may be employed. Copper has the great advantage for this purpose 105 that it is actively toxic to all the fungi and

particularly to the fungi causing dry rot. The toxicity of copper for this purpose is very great, and the amount of the copper salt which need be used is correspondingly small. A minimal amount of any copper salt in wood or other fiber will wholly prevent the growth of the dry rot organism. Copper salts, in and of themselves, are not suitable for preserving wood, partly because the amount required for a tie in the absence of any other preservative is very large and partly because they are usually fairly soluble in permeating moisture, so that an impregnation with copper does not last long. Of course any copper salt which is carried into the fiber by water can be removed by water again.

By dissolving a minimal amount of copper salt in an asphalt or asphalt-like oil, a composition is obtained which, in addition to the physical advantages of the asphalt, has the very great and positive advantage of the fungicidal properties of the copper. In such an impregnating composition it is not necessary to use more than a per cent. or so of the copper compound and much less will frequently suffice.

While many kinds of asphalt and asphalt-like bodies may be employed under the present invention, I prefer the asphalt-like compositions derived in distilling certain kinds of petroleum such as the Oklahoma petroleum. The residuum from other kinds of petroleum having a paraffin base, is not so suitable unless it be previously treated by oxidation, sulfurizing or any other way to convert it into an asphalt-like mass, such as the well known "byerlyte." Untreated paraffinic petroleum residuum is not nearly so well suited for this purpose, and particularly when the treated wood is to be used for ties or lumber purposes. Such a paraffinic residuum has of course considerable lubricating activity and spikes and nails do not hold well in the wood treated therewith. With the asphaltic compositions used under the present invention on the other hand, the treating agent gives an additional holding power to the wood. This is of course a great advantage for most purposes.

Asphaltic compositions of the nature of these stated contain practically no volatile or soluble matter and there is no loss of impregnating agent by volatilization, or by leaching. The impregnating agent is therefore perfectly permanent in the tie or other wood article. Being practically inert they do not "tender" or weaken the wood fiber. These asphaltic bodies while more viscous and stiffer in character than the creosotes and dead oils, which is an advantage after impregnation, nevertheless upon heating become quite thinly fluid and are easily used for impregnating purposes. While such asphaltic bodies are substantially inert, never-

theless as a rule on exposure to air they suffer a slight thickening or hardening action. As a result of this the exterior portions of impregnant in a tie or pole harden up a little thus sealing in the rest of the 70 impregnant which of course remains in an unchanged condition. In a heated and thinly liquid condition the penetrating properties of the asphaltic oil are very satisfactory, as it requires but little time to 75 reach the interior of the wood and produce a thorough impregnation. After cooling, while not thin enough to permit capillary withdrawal by the soil, etc., the material is nevertheless fluent enough to permit its 80 entering in freshly formed checks or checked cracks, thus aiding in the waterproofing qualities and preventing water from entering the wood as it ages. In the wood these asphaltic oils are absolutely permanent, not changing with time except for the slight superficial hardening referred to, a 85 property which is advantageous. The asphaltic oil is practically odorless and is not disagreeable or dangerous to handle as are 90 creosote and dead oil. It may be handled with impunity. Different samples of asphaltic oil also run very uniform in composition and quality. Commercial creosotes and dead oils are very variable in quality 95 and it is difficult to obtain two consignments which are alike.

As a suitable copper compound for solution in the asphalt may be used a copper oleate or resinate, or a mixture or compound 100 of resinate and oleate. For instance, copper carbonte, hydrate or oxid may be heated with rosin and oleic oil or red oil. In a typical recipe, about 5 pounds of copper carbonate, 10 to 12 pounds of red oil, and 105 3 or 4 pounds of rosin may be heated in a suitable vessel at a temperature of about 140° C. until the oily mass is saturated with dissolved copper. With copper carbonate 110 considerable effervescence occurs and the mass is apt to froth badly so that it is desirable that the vessel employed have ample capacity. It is better to add the copper carbonate, where this compound is used, in successive small portions. After the copper 115 has gone into solution as an organic salt, the oily composition produced is gradually mixed with any desired quantity of asphaltic oil. Or the asphaltic oil may be gradually added to the oily copper composition in the same vessel. A content of 120 about 1 per cent. of copper in the asphaltic oil is a suitable strength for most purposes. For the sake of convenience it is frequently desirable to make stronger solutions of the copper carbonate in the asphaltic oil and use these for treating larger quantities of asphaltic oil to obtain solutions of the desired strength for use. Where the asphaltic oil, as is frequently the case is a solvent of 125 130

copper, the hydrate or carbonate of copper or other toxic metal may be dissolved directly in the oil.

Other metallic carbonates, oxids, or hydrates may be used in lieu of the copper compounds, but are usually no more desirable. They may, however, be used for special purposes. Zinc compounds are suitable though not as active in preventing dry rot 10 as the copper compounds. Arsenic may be used in connection with, or substituted for the copper compounds where an actively poisonous action is desired as in the case of piles to be made teredo proof. Chlorids, 15 bromids, iodids, sulfocyanids, etc., of arsenic may be employed, as these compounds are soluble in oily solvents. Antimony compounds are less suitable.

The asphaltic oil containing the toxic mineral compound may be entered into the fiber in any of a number of different ways. For instance, the toxic oil may be simply heated in a vessel and the wood dipped for the requisite length of time. Impregnation 20 may be aided by the use of pressure such as steam pressure or air pressure, or by vacuum. With old and seasoned wood, the wood may be previously steamed or treated with hot water to open up the pores, the 25 moisture being subsequently removed as by the use of vacuum. This steaming, however, is rarely to be recommended as any residual moisture in the pores of the wood interferes with the entrance of oily bodies 30 such as the toxic asphaltic oil. A suitable method of impregnating is to place the air dried wood in a suitable vessel capable of withstanding pressure and produce a pressure therein of about 5 atmospheres by the 35 use of air or steam. The toxic asphaltic oil is then run in the treating vessel under a pressure of say, about 15 atmospheres. After removal of the wood from the oil and the release of pressure, the contained air or 40 steam under pressure in the pores, forces its way outward carrying with it the bulk of the oil used and leaving merely enough to wet and impregnate thoroughly the fibers of the wood. This treatment gives a wood 45 having its normal porosity but with each fiber covered, impregnated and protected by the toxic oil. In this method where relatively a small amount of impregnating oil is employed the presence of the toxic agent 50 dissolved in such oil is particularly valuable. The oil in this treatment must be heated sufficiently to make it thinly liquid. Instead of this method of entering the oil a vacuum may be first applied to the wood 55 and then the toxic oil introduced. This results in a very thorough penetration of the oil. Or the wood may be treated in the presence of the oil alternately under vacuum and under pressure. However, for most 60 purposes simply heating the wood in the

oil to a temperature around 100° C. is sufficient as this vaporizes the moisture in the pores and allows the toxic oil to take its place.

The copper compound being entirely dissolved in an oily solvent does not injure iron treating cylinders, pumps, pipes or other mechanical elements as do water solutions of copper salts. The toxic oil is entirely inert as regards metallic surfaces. 70

The toxic oil may of course be used in the form of an emulsion with watery impregnators such as corrosive sublimate, zinc chlorid, etc., but there is little advantage in this. Asphalt oils of the character contemplated in the present invention are very cheap and their preservative action when made toxic in the manner described is so much superior to that of the watery solutions of mineral salts that it is not usually 80 necessary or desirable to let them down by forming emulsions with such solutions of preservative substances.

While the described process and composition may be usefully employed for impregnating other vegetable fibrous material than wood, as in making "tar paper" for roofing, siding and the like, in making "tarred" rope, etc., yet I regard the present invention as more particularly applicable to treating wood and lumber intended 90 for ties, poles and structural purposes. 95

The toxic oil so prepared may of course be admixed with any desired amount of petroleum, creosote, dead oil, or other impregnator if desired, or with mixtures of these substances. This is, however, not in general desirable since these bodies do not have the peculiar properties of the toxic asphaltic oil. Similarly, emulsions of zinc 100 chlorid, copper sulfate, etc., may be admixed with the toxic oil, but this addition is not generally desirable. The woody fiber may be impregnated with a watery solution of a fireproofer if desired, and then given 105 a subsequent coating impregnation with the toxic oil thereby sealing in said watery fire-proofing material and protecting it against solution and volatilization. 110

Where the asphaltic oil used is not sufficiently viscous when cold, tarry or asphaltic bodies may be added to heighten the viscosity. 115

What I claim is:—

1. The process of preserving wood which 120 comprises dissolving a toxic mineral body in an asphaltic body of a fluent but viscous nature and impregnating wood with the composition so formed.

2. The process of preserving wood which 125 comprises dissolving a toxic mineral body in an asphaltic oil of a fluent but viscous nature and impregnating wood with the composition so formed.

3. The process of preserving wood which 130

- comprises dissolving a toxic mineral body in an asphaltic petroleum residuum of a fluent but viscous nature and impregnating wood with the composition so formed.
- 5 4. The process of preserving wood which comprises dissolving a copper compound in an asphaltic body of a fluent but viscous nature and impregnating wood with the composition so formed.
- 10 5. The process of preserving wood which comprises dissolving a copper compound in an asphaltic oil of a fluent but viscous nature and impregnating wood with the composition so formed.
- 15 6. The process of preserving wood which comprises dissolving a copper compound in an asphaltic petroleum residuum of a fluent but viscous nature and impregnating wood with the composition so formed.
- 20 7. As a new article of manufacture, wood having incorporated therewith an asphaltic
- body carrying a dissolved mineral toxic agent.
8. As a new article of manufacture, wood having incorporated therewith an asphaltic 25 body carrying a dissolved copper compound.
9. As a new article of manufacture, wood having incorporated therewith an asphaltic petroleum residue carrying a dissolved mineral toxic agent.
10. As a new article of manufacture, wood having incorporated therewith an asphaltic petroleum residue carrying a dissolved copper compound. 35

In testimony whereof, I affix my signature in the presence of witnesses.

CARLETON ELLIS.

Witnesses:

NATHANIEL L. FOSTER,  
FRANCES I. NEWMAN.